

# UNITED STATES PATENT OFFICE.

HANS GOLDSCHMIDT AND HANS BIEWEND, OF ESSEN-ON-THE-RUHR, GERMANY,  
ASSIGNORS TO GOLDSCHMIDT THERMIT COMPANY, OF NEW YORK, N. Y., A  
CORPORATION OF NEW YORK.

## PROCESS FOR IMPROVING THE PROPERTIES OF INGOT-IRON AND THE LIKE.

1,122,272.

Specification of Letters Patent. Patented Dec. 29, 1914.

No Drawing.

Application filed May 31, 1912. Serial No. 700,785.

*To all whom it may concern:*

Be it known that we, HANS GOLDSCHMIDT and HANS BIEWEND, subjects of the King of Prussia, and residents of Essen-on-the-  
5 Ruhr, in the Province of the Rhine, Germany, have invented certain new and useful  
Improvements in Processes for Improving  
the Properties of Ingot-Iron and the like, of  
which the following is an exact specification.  
10 A process of manufacturing homogeneous  
metl castings has been previously proposed  
in which heat produced by an aluminothermic  
reaction was made to act upon certain  
points of a casting. More particularly this  
15 process was intended to be carried out in  
such a manner, that by introducing an aluminothermic  
mixture into the solidifying  
head of an ingot, the latter was to be kept  
liquid for a longer time so as to make the  
20 ingot capable of receiving further liquid  
steel. Now practice has shown that although  
certain parts of the ingot can be heated and  
kept fluid by this process it is impossible to  
remove a great number of disadvantages by  
25 same. So for instance frequently the case  
may arise that an ingot contains a shrinkage  
hole or cavity which is not tapering off in  
a regular manner but shows displacements  
or interruptions. If now the heat, produced  
30 according to the previously known process  
by an aluminothermic reaction, would be  
allowed to act upon the head of the ingot,  
only the upper part of the cavity inter-  
rupted by displacements, but not the lower  
35 part of such hole would be made accessible  
to the liquid metal to be further filled in.  
Furthermore, many places of the ingot fre-  
quently show blisters as a consequence of the  
inclusion of gases. These hollow spaces  
40 cannot at all or can only partly be removed  
by allowing the heat arising from an alu-  
minothermic reaction to act at a certain  
spot and more particularly at the head of  
the ingot.

45 Now a long series of experiments has  
shown that by allowing the heat, produced  
by an aluminothermic reaction to act at cer-  
tain spots of a casting a thorough improve-  
ment of the properties of the ingot cannot  
50 be obtained because only a local action by  
means of fusion or repeated liquefaction is  
obtained by this process. Further experi-  
ments have shown that the disadvantages  
above-mentioned can not only be avoided,

but that also a number of important advan- 55  
tages can be obtained by making use not of  
a local thermal effect only, but of a mechani-  
cal effect of the aluminothermic mixture.  
If namely a certain time after the casting is  
finished the aluminothermic mixture is in- 60  
troduced into the solidifying ingot, the in-  
terior of which is still fluid, in such a man-  
ner that the aluminothermic mixture comes  
down as far as possible to the bottom of the  
ingot mold, one immediately observes that 65  
the metal in the interior of the ingot is  
brought into a bubbling and whirling mo-  
tion, which extends up to the surface. By  
this mechanical motion which is aided by  
the rapid rise of the light slag all blisters or 70  
gas bubbles inclosed or retained in the in-  
terior of the ingot are forced up to the sur-  
face. Furthermore, all the segregations  
which always separate out in the longitudi-  
nal axis of an ingot and likewise particles of 75  
slag, which accidentally have come into the  
ingots, are in the same manner brought to  
the surface. How perfectly the removal of  
gas, segregations and the like is effected may  
be seen from the fact that immediately after 80  
the reaction the contents of the ingot mold  
shrink for a considerable amount.

The new recognition is that all the factors  
acting unfavorably upon the properties of  
the ingot are eliminated by producing a 85  
whirling motion directed from the bottom to  
the surface within the solidifying ingot the  
interior of which is still fluid. This whirling  
motion is preferably caused by introducing  
90 an aluminothermic mixture as described  
above, as aluminothermic mixtures all those  
mixtures being understood, which are com-  
posed of one or more metal oxids and alu-  
minum or other reducing metals, by the re-  
action of which heat is produced.

95 The bubbling and whirling motion which  
is the cause of improving the qualities of  
the cast ingot can not only be produced by  
the introduction of an aluminothermic mix-  
ture but also by various other means for in-  
stance with the aid of explosives the speed  
of explosion of which is particularly small,  
or by means of gases introduced under high  
pressure, which do not dissolve within the  
ingot metal, or finally by producing electric 100  
currents within the liquid metal. Now, in  
order to obtain the result that the whirling  
motion and its effects extend throughout the

ingot, it has proved necessary that for instance the box or the like containing the alumino-thermic mixture, is pushed down as far as possible to the bottom of the mold.

5. After the reaction is finished and the steel rod by means of which the box has been introduced has been withdrawn, the liquid iron or steel sinks down in the ingot mold. Then the latter is again filled up 10 with liquid steel or the like metal from the ladle as quickly as possible, the steel being cast from above into the mold in such a manner that the surface equals the level of the crust which has been formed at the 15 face of the mass. Hereafter the covers are laid upon the molds which then remain on their places till the ingots are perfectly solidified.

The advantages above described are apparent for instance if low carbon steel without silicon in form of ingots is rolled to sheet metal. The practice has shown that the waste of the sheet rolled from material treated according to the above process is 20 limited to about 0.3%, whereas the waste in the manufacturing of sheet made of ordinary ingots is much higher, in some cases even fifty times and more. Moreover with the process described, besides the advantages 25 above-mentioned some other advantages are obtained which consist in an essential refining action on the material. It is however not possible to give numerical values for them in the same manner as 30 above.

What we claim is:

1. A process for improving the properties of metals cast in ingots which consists in producing in the fluid interior of the 35 metal body shortly before solidification a

whirling or bubbling motion directed from the bottom to the surface.

2. A process for improving the properties of metals cast in ingots which consists in producing in the fluid interior of the metal 45 body shortly before solidification a whirling or bubbling motion directed from the bottom to the surface and extending throughout the ingot body.

3. A process for improving the properties 50 of iron, steel and the like cast in ingots which consists in producing in the fluid interior of the iron and the like material a whirling or bubbling motion directed from the bottom to the surface and extending 55 throughout the ingot body.

4. A process for improving the properties of iron, steel and the like cast in ingots which consists in introducing an alumino-thermic mixture into the fluid metal of the 60 ingot thereby producing a whirling or bubbling motion in the interior of the ingot mass, and extending throughout the ingot body.

5. A process for improving the properties 65 of iron, steel and the like cast in ingots which consists in introducing an alumino-thermic mixture into the fluid metal down to the bottom of the latter, thereby producing a whirling or bubbling motion in the 70 interior of the mass directed from the bottom to the surface.

HANS GOLDSCHMIDT. [L. S.]  
HANS BIEWEND. [L. S.]

Witnesses as to Hans Goldschmidt:

JESSIE E. POST,  
Wm. C. CURITS.

Witnesses as to Hans Biewend:

HELEN NUFER,  
ALBERT NUFER.